

# United States Patent Office

3,240,797

Patented Mar. 15, 1966

1

3.240.797

**3,240,791**  
**BIS(SULFATOETHYL) SULFOXIDE SALTS**

DISUBSTITUTED, SOLOXIDE SALTS  
Donald J. Gale, Spartanburg, S.C., assignor to Deering  
Milliken Research Corporation, Spartanburg, S.C., a  
corporation of Delaware  
No Drawing. Filed Dec. 31, 1959, Ser. No. 863,217  
2 Claims. (Cl. 260—458)

corporation of Delaware  
No Drawing. Filed Dec. 31, 1959, Ser. No. 863,217  
2 Claims. (Cl. 260—458)

This invention relates to modified cellulose yarns and fabrics having an improved configurational memory, and to methods and chemicals used in making the same. More particularly the invention relates to modified cellulose yarns and fabrics having an improved tendency to return to an original flat, creased or similar configuration when washed and thereafter dried.

It is well known that fabrics can be formed which have a tendency to return to a predetermined configuration after washing. For example, by applying certain resins to fabrics and curing the resin while the fabric is in a flattened condition, one can obtain a fabric that, when allowed to dry in a flat condition, has a pressed appearance and requires no ironing. In a similar manner, one can form "permanent" pleats in a fabric so that the pleats are not removed by washing. The fabric dries flat between creases, and no ironing of the fabric is required. Any such fabric, or yarns capable of resulting in such fabrics, are referred to in this specification as "flat drying" and it will be understood that this term is employed broadly to include any textile material which normally requires no ironing, pressing or the like for a satisfactory appearance.

These fabrics which obtain their flat drying properties as a result of resin application, commonly referred to in the trade as wash and wear fabrics, have one or more of the following disadvantages: (a) lack of durability, (b) odor formation, (c) chlorine retention, (d) loss of strength and (e) susceptibility to wrinkling when wet. On account of the latter disadvantage, these fabrics must be drip dried since they given a low degree of recovery from creases when wet. The inconvenience of drip drying is well known.

Other treatments include the cross linking of cellulose by means of dichloropropanol or epichlorohydrin in the presence of strong alkali. Such treatments inevitably were accompanied by severe losses in tensile and tear strength.

Another way for producing like effects is to treat the fabric with divinyl sulfone and alkali according to U.S. Patent 2,524,399. The disadvantage of this last treatment is that the divinyl sulfone is a very toxic and lacrimatory material, that the divinyl sulfone is subject to polymerization upon exposure to the alkaline solution. Therefore when the fabric is treated with the solution of divinyl sulfone and alkali, the divinyl sulfone reacts partially with the cellulose and polymerizes partially. All of the abovementioned treatments are also defective in that the cotton so treated suffers from alkaline oxidation.

Fabrics woven of certain synthetic materials, such as glycolterephthalate fibers, also display flat drying qualities but such fabrics likewise have several inherent disadvantages. For example, flat drying polyester fabrics are expensive, have a tendency to collect static electricity, and, if formed from staple fibers, generally display a tendency to pill badly. In addition, polyester fabrics have a low moisture absorptivity so that they feel cold to the touch and are incapable of absorbing perspiration from the body. Still another disadvantage is that they become dingy after repeated washings and cannot be readily bleached.

Flat drying fabrics prepared by other methods general-

2

ly must be "drip dried"; that is, they must be hung immediately after they are withdrawn from the wash and before they are wrung. It is, therefore, inconvenient to drip dry even a single item of clothing and almost prohibitive to drip dry large quantities of clothing.

Cross linking agents which have been used in treating cellulosic fibers to make flat drying fabrics have not been as chemically reactive as desirable, and in many cases not as water soluble as desirable, and in some cases have been rather volatile, at least under reaction conditions so that they tend to escape into the room. Therefore, special ventilating procedures and apparatus are required for handling such materials. Moreover, it would be desirable to reduce or eliminate the "wet sliciness" that seems to be inherent in fabrics treated with some cross linking agents.

An object of the present invention is to obtain reagents and procedures for preparing flat drying fabrics that overcome the many disadvantages of the resin treated fabrics.

20 Another object of the invention is to obtain such reagents that are more chemically reactive than other cellulose cross linking agents, so that the reaction can take place in a short time thereby facilitating continuous operations.

25 Still another object is to obtain such reagents which are more specific in their cross linking reaction with cellulose so that there will be fewer side reactions.

Still another object of the invention is to obtain such reagents that are soluble in water so they can be readily

used in solution instead of in emulsion form. Still another object of the invention is to obtain such reagents that have practically no volatility and therefore do not create any ventilation problems in the mill.

Another object of the invention is to produce flat drying cellulosic fabrics that do not have to be drip dried but will retain their configurational memory as long as they are wet and therefore can be put through a roller or a centrifugal wringer before they are hung.

Other objects and advantages of the invention will be apparent from the following description:  
The invention resides in the discovery of certain reagents which are novel compositions of matter and which are effective in imparting flat drying properties to cellulosic fibers, and also in the use of such reagents in treating cellulosic fibers. According to the invention cellulosic fibers, yarns or fabrics while in a swollen condition are reacted with a cross linking agent represented by one of the following formulae:

$$X[CHR^1-CHR^2-O-SO_3-Y]_2$$

50 or



55 in which

$R^1$  and  $R^2$  are hydrogen or saturated alkyl groups having 1 to 3 carbon atoms such as methyl, ethyl or propyl,  $Y$  is hydrogen or any metal ion or nitrogen base that produces a soluble reagent.

$X$  is  $-\text{SO}_2-$  or  $-\text{O}_2\text{S}-\text{R}-\text{SO}_2-$

The compound  $X\{CHR^1-CHR^2-O-SO_3-Y\}_2$  are of particular interest because they may be in the form of salts and therefore nonvolatile and easy to handle in the mill. Such compounds are also water soluble.

In the formula for this group of compounds, R may be any of several groups of radicals, as follows:

(a) A saturated aliphatic divalent radical, said radicals consisting essentially of from 1 to 10 carbon atoms, hydrogen, 0 to 4 oxygen atoms, 0 to 2 sulfur atoms, and metal ions (or nitrogen base ions) in amount not ex-

ceeding that necessary to replace carboxylate and sulfonate acid hydrogens. The oxygen in the saturated aliphatic radical is present in ether, sulfonate or carboxylate groups. The sulfur is present in thioether or sulfonate groups; or

(b) Cycloaliphatic radicals consisting essentially of 4 to 7 carbon atoms, 0 to 3 oxygen atoms, 0 to 1 sulfur atoms, and metal ions (or nitrogen base ions) in amount not exceeding that necessary to replace the carboxylate and sulfonate acid hydrogens. The oxygen of the cycloaliphatic radical is present in sulfonate, ether or carboxylate groups. The sulfur is present in thioether or sulfonate groups. Moreover, the sulfonate groups of the radical X are attached directly to —CH— groups in the cycloaliphatic ring; or

(c) The aromatic groups meta or para phenylene, meta or para phenylene substituted with hydrocarbon groups having 1 to 3 carbon atoms, or



where the groups Z in the aggregate consist essentially of hydrogen, 0 to 3 carbon atoms (present as the alkyl groups methyl, ethyl or propyl), 0 to 2 sulfur atoms, and 0 to 6 oxygen atoms, the oxygen and sulfur being in the form of sulfonate groups. The valence bonds \* are linked to the sulfone groups of the radical X. Moreover, there are no two  $-\text{SO}_2-$  groups that are ortho to each other on the naphthalene ring whether from the sulfone or from any sulfonate substituents.

The reagent represented by the first general structural formula given above may be a metallic (or nitrogen base) salt of the sulfuric ester. Any metal or nitrogen base that produces a soluble reagent may be used to supply the cation. The alkali metal salts such as lithium, sodium, and potassium are readily available and therefore acceptable. The alkaline earth metal salts such as barium, calcium, and magnesium are also suitable (except that barium and calcium should not be used when a sulfonate group is present because of insolubility problems). However, other metallic ions that produce water soluble reagents and therefore also lend themselves to being used include lead, tin, zinc, iron, nickel, cobalt, ammonium, and manganese.

The choice of nitrogen bases is also very broad. Even very weak bases such as aromatic and aliphatic amines including aniline, methyl and ethyl amines can be used. Of course, the strong quaternary hydroxide amines are satisfactory. These include benzyl trimethyl ammonium hydroxide, tetramethyl ammonium hydroxide, trimethyl phenyl ammonium hydroxide and others.

As will be explained later, it is believed that the cross linking agents of the present invention react with the hydroxyl groups of the cellulose molecule through the medium of the sulfated ethyl group. The sulfone group  $-\text{SO}_2-$  is believed to be important in imparting the desired activity and specific reactivity with cellulose hydroxyls desired in the sulfated groups. It follows also that the character of the group R is of secondary importance, the object merely being to select groups which will not interfere with the reaction of the sulfated ethyl groups with the cellulose hydroxyls.

The radicals R are classified under three main headings: 65

- (a) Saturated aliphatic radicals,
  - (b) Cycloaliphatic radicals, and
  - (c) Aromatic groups.

Taking up first the group (a) saturated aliphatic radicals, it is desirable to avoid groups such as alcohol ( $-\text{OH}$ ) and nitrogen, ( $-\text{NO}_2$ ,  $\text{NH}_2$ ) groups. However, oxygen and sulfur-containing groups such as ether, thioether, sulfonate, and carboxylate groups are permissible. In order to exclude unduly complicated radicals

which may interfere with the cross linking reaction through steric hindrance or insolubility, the number of such groups is generally restricted so that the total number of oxygen atoms is not greater than two, the number of sulfur atoms is not greater than two, and the total number of carbon atoms in the group R is restricted to one to ten inclusive. In instances where sulfonate and carboxylate groups are present, the acid hydrogens may be partly or entirely replaced with weak or strong positive basic ions.

Aliphatic radicals that may be included in the cross linking agents of the invention include:



The second classification of the radical R is the cycloaliphatic radicals. It is intended to include within this class compounds in which the sulfone groups of the group X are attached directly to the ring, i.e., directly to a  $-\text{CH}-$  group of such ring.

As in the case of the aliphatics, the character of the group R is only of secondary importance. The object is to avoid interfering with the reactivity of the sulfated ethyl group. Therefore, the group R is generally restricted to those having 4 to 7 carbon atoms. Although oxygen and sulfur may be present, such elements would be in the form of ether, sulfonate, carboxylate or thioether groups. Moreover, the total number of oxygen atoms in the cycloaliphatic radical is from 0 to 3, and the total number of sulfur atoms is 0 to 1. The following cycloaliphatic radicals are examples of those which may be present in the group X of the cross linking agents of the present invention.



In addition to the 4 to 7 carbon atoms, 0 to 3 oxygen atoms, and 0 to 1 sulfur atoms which make up the cyclo-aliphatic radical R, any carboxylate or sulfonate group may have its acid hydrogen partly or wholly replaced by a strong or weak metal ion.

The third kind of group R is aromatic. The aromatic group may be phenylene (or substituted phenylene), or it may have a naphthalene base. In this case also, the number and type of substituents are restricted to exclude those that may interfere with the desired reaction. The substituents on the naphthalene group are preferably no

more than one hydrocarbon group having 1 to 3 carbon atoms, and such naphthalene groups having no more than two sulfonate substituents. Recognizing that  $-\text{SO}_2-$  groups of the radical X will be attached to the naphthalene groups and that sulfonate substituents (if present) may supply additional  $-\text{SO}_2-$  groups, it is desirable that there shall be no  $-\text{SO}_2-$  substituents that are ortho to each other on the naphthalene nucleus. Examples of radicals R that fall within the category of aromatics are:



The following are examples of specific compounds that may be used as cross linking agents:



Compounds in which the group X is the sulfone  $-\text{SO}_2-$  may have a tendency to react within the molecule to form an eight membered ring structure. Although this group of compounds has the desirable properties of reactivity with the hydroxyl groups of cellulose, they are generally somewhat less soluble and more volatile than the acid and salt forms discussed above. The resulting cyclic compound has the following structure:



Specific examples of such a compound are:



or



The process can be satisfactorily performed on yarns or fabric containing either natural cellulose fibers, regenerated cellulose fibers and/or chemically modified cellulose fibers having a portion of the hydroxy groups thereof blocked by ester or ether groups, provided that the fibers retain their general form when wetted with water. Examples of materials of the latter type which can be employed include yarn or fabrics composed of

cellulose acetate or methyl cellulose fibers. Generally, however, the cellulosic fibers should have an average of at least 1.8 free hydroxy groups per glucose unit. Cellulosic materials having a smaller number of free hydroxy groups do not give satisfactory results even though, in the case of cellulose esters, the ester groups might theoretically be removed by hydrolysis during the cross linking reaction. Satisfactory results can also be achieved with yarn or fabrics partially composed of other than cellulosic materials and this is particularly true where the non-cellulosic fibers have some known flat drying properties of their own. For example, the flat drying tendencies of yarn spun from a mixture of glycol-terephthalate fibers and cotton fibers can readily be increased by the process of this invention, even if the percentage of cotton fibers is as small as 10%. Even when the non-cellulosic fibers display no flat drying properties, yarn and fabrics containing the same can be caused to display flat drying properties by the present process if the yarn or fabrics contain at least about 40% by weight of cellulosic fibers.

It is believed that the reaction between the cross linking agent and the cellulose molecule takes place according to the following equation:



Apparently, the reaction with the cellulose proceeds through a substitution of the alkali cellulose for the sulfato group which is split off from the ethyl radical forming a cellulose ethyl ether. This reaction takes place without the formation of intermediate vinyl sulfone and has the specific advantage over the reaction of the vinyl sulfone with the cellulose in that the alkali which is present in the cellulose micelle during the reaction with the sulfato ethyl sulfone is neutralized by the sulfato radical which is split off from the ethyl group, thus avoiding alkali damage to the cellulose. The cellulose is first treated with an aqueous solution of the cross linking agent and dried and then immersed in a strong solution of alkaline medium, preferably an aqueous alkaline solution. Suitable alkaline materials are the alkali metal hydroxides such as sodium hydroxide, potassium hydroxide, the alkali metal sulfides such as sodium sulfide, quaternary ammonium hydroxides such as benzyl trimethyl ammonium hydroxide, tetramethyl ammonium hydroxide, or trimethyl phenyl ammonium hydroxide. The amount of strong alkaline material present during the cross linking reaction is at least two equivalents per mole of the cross linking agent in addition to any that may be needed to neutralize acidic hydrogen atoms in the molecule. For example, if the agent contains a sulfonic acid or a carboxylic acid group, the amount of alkali would be increased correspondingly.

A sufficient amount of cross linking agent should be used in order to provide enough cross linkages to give the degree of cross linking that will produce a noticeable amount of flat drying. Due to the high chemical efficiency of these cross linking agents, only a very small amount is required. Generally at least 0.005 mole per anhydro-glucose unit is sufficient. Preferably a somewhat larger quantity of 0.01 mole of cross linking agent per anhydro-glucose unit is used. Larger amounts can be used, though with some sacrifice of flexibility and strength of the fibers (as well as economy). Hence, I prefer to keep the amount of cross linking agent below 0.05 mole per anhydro-glucose unit.

The manner of applying the agent and the strong alkali to the cellulose is also subject to wide variation. In many cases, it is preferred first to place the cross linking agent on the fabric as an aqueous solution, then dry the fabric and apply just enough strong alkali to meet the requirements set forth above. In this way, there is almost no leaching out of the cross linking agent into the alkali

solution. Both the treating agent solution and the alkali solution can be applied by conventional padding or by spraying techniques. In one process the treated fabric containing the agent is passed downwardly through the nip between the two rubber covered rollers and the alkaline solution is also fed into the nip in just the right amount to saturate the fabric and be carried through the nip with the fabric. If leaching of the agent from the cloth by the aqueous caustic is or becomes a problem, salt such as sodium chloride may be desirable in the aqueous alkali to reduce the solubility of the agent therein.

It is not necessary to put the cross linking agent on the fibers first. The alkaline material may be applied first or the two may be applied simultaneously.

Substantial advantages of the invention arising out of the solubility of the cross linking agent in water are its low volatility and its high selective reactivity for cellulose. The greater reactivity and selectivity make it possible to carry out the reaction in a shorter time and thereby make continuous operation possible. Because of the lower volatility of the acid and the salt forms, the material is easier to handle in the plant and ventilation problems are greatly simplified. The solubility of the agents in water not only avoids the problem of preparing emulsions, but also greatly improves the penetration and uniform distribution of the treating agent through and over the cloth or yarn, as the case may be.

The temperature of the reaction and the time of reaction are mainly interdependent. The reaction may, if desired, be carried out as low as room temperature, in which case a reaction time of 30 minutes may be expected. If the material is heated slightly, say to 40° C., the reaction will be completed in as little as 30 seconds. If still a higher temperature is maintained, say 95° C., reaction is complete in only a few seconds. Some heat is generated from the reaction itself and this effect alone may account for a temperature rise in the material from 40° C. to about 60° C.

The cross linking reaction tends to fix permanently the configuration of the fabric or yarn as that prevailing during the reaction. In other words, if one desires a fabric that will have a flat and pressed appearance after washing, it is necessary that the fabric be retained in a flat and slightly tensioned condition during the cross linking reaction. This can be accomplished by conducting the reaction while the fabric is in a tenter frame. Of course, if it is desired that the fabric display permanent pleats or the like, then it is necessary that the cross linking reaction be conducted while the fabric is in a pleated condition.

Following the cross linking reaction, the fabric or yarn should be thoroughly scoured employing any suitable detergent. This serves mainly to remove reaction by-products such as sodium sulfate and also to remove any excess alkali and sodium chloride that may be present.

The cross linking agents can be prepared in the following manner when the group X is  $-\text{SO}_2-$



This reaction is the well known addition reaction of hydrogen sulfide to ethylene oxide or substituted ethylene oxide to produce bishydroxyethyl sulfide. The latter compound is then oxidized using, for example, hydrogen peroxide or potassium permanganate as an oxidizing agent to produce bishydroxyethyl sulfones  $\text{O}_2\text{S}[\text{CHR}^1-\text{CHR}^2-\text{OH}]_2$ . Finally, the bishydroxyethyl sulfones are treated with sulfuric acid to form bisulfatoethyl sulfones



The bisulfatoethyl sulfones may be applied directly to the cellulose fibers (in which case, as explained above, additional quantities of alkali will be required) or they may first be neutralized with an alkaline material to replace the

acidic hydrogen of the sulfuric acid group with a metallic or equivalent ion.

Instead of treating the cellulose with the acid sulfatoethyl compound, any salt of such acid with a weak or 5 strong base may be used. By reacting the bisulfatoethyl sulfone acid with any metal oxide or hydroxide from the group described above (in defining the symbol Y), the bisulfatoethyl sulfone salt of such a metal may be formed. If the metal oxide or hydroxide is insoluble it should be 10 used in finely divided form, giving enough time, preferably with some heat, for the reaction with the acid compound to take place.

Another way of forming the bisulfatoethyl sulfone salts of metals is to pass a solution of the corresponding acid through an ion exchange bed containing the metallic ion that is to be substituted for the acidic hydrogen.

The sulfatoethyl sulfones in the acid and salt forms are 15 stable compounds and, therefore, can be isolated and stored for future use or they can be used immediately in 20 the solutions in which they are first prepared.

The cyclic compounds



25 can be made by heating the acid form of the corresponding bisulfatoethyl sulfone with the elimination of  $\text{H}_2\text{SO}_4$ .

The cross linking agents in which the group X is 30  $-\text{SO}_2-\text{R}-\text{SO}_2-$  may be formed by similar reactions using a bis mercaptan instead of  $\text{H}_2\text{S}$ .

$\begin{array}{c} \text{O} \\ | \\ \text{CHR}^1-\text{CHR}^2 + \text{HS}-\text{R}-\text{SH} \longrightarrow (\text{HO}-\text{CHR}^1-\text{CHR}^2\text{S})_2\text{R} \end{array}$   
The intermediate product is oxidized with peroxide or 35 permanganate as described before to form the sulfone  $(\text{HO}-\text{CHR}^1-\text{CHR}^2-\text{SO}_2)_2\text{R}$ . The latter compound is then treated in a manner similar to the bishydroxyethyl sulfone mentioned above, i.e., with sulfuric acid or  $\text{SO}_3$  to form the corresponding bisulfatoethyl sulfone, which 40 may be used as such or may be converted to any of the metal or nitrogen base salts described above.

The compounds in which the group X is



45 wherein the group R is aromatic and the two sulfones are attached directly to the aromatic ring, can be readily prepared by the following procedure:

The compound



50 is prepared by known procedures by treating benzene with chlorosulfonic acid. The material is then treated with sodium sulfite in an aqueous solution of sodium hydroxide to form the compound



55 The material so formed is then treated with



60 while refluxing in aqueous solution to form the compound



65 70 which is treated with 30% fuming sulfuric acid according to the procedure described above for the hydroxyethyl sulfones.

75 One aspect of the present invention is directed to the combined application of resin materials of the class to be described more fully hereafter and the cross linking agents

set forth above. Such resins, when used alone, at least in amounts sufficient to impart flat drying characteristics, have the undesirable characteristic of imparting poor hand to the fabric with a tendency to become discolored when repeatedly bleached with household bleaches. Furthermore, the resin tends to be removed from the fabric after a number of launderings. If the amount of resin is reduced, then the dry crease resistance as normally imparted by the resin treatment is decreased or even lost.

By combining the resin treatment with the cross linking agent of the present invention, however, it has been found that the two reagents exert a synergistic action upon each other so that by reducing the amount of resin, the normal undesirable properties of resin treatment are minimized, but the flat drying characteristics are retained.

The resinous materials which can be employed and which will hereinafter be referred to simply as "textile resins" are low molecular weight (less than 1,000), water soluble, acid or acid salt catalyzed materials which are thermosetting at least in the presence of cellulosic materials as above defined. The largest class of resins within this group comprises the aminoplast resins formed by reacting compounds such as urea and melamine with formaldehyde, and specific examples of resins within this class include urea formaldehyde resins such as the resin commercially available from Rohm & Haas under the trade name of "Rhonite 610"; methyl ethers of urea formaldehydes such as the resin sold by Rohm & Haas under the trade name of "R-2 Resin"; acrolein urea formaldehyde resins; cyclic ethylene urea formaldehyde resins such as the resin sold by E. I. du Pont under the trade names of "Zeset" and the resin sold by Rohm & Haas under the trade name of "R-1 Resin"; trimethylol acetylene diurea; tetramethylol acetylene diurea; melamine formaldehyde resins such as the resins sold by Monsanto under the trade name of "Resloom H.P." and "Resloom L.C."; methylated melamine formaldehyde resins such as the resin sold by American Cyanamid under the trade name of "M-3 Resin"; or the resin sold by Monsanto under the trade name of "M-75 Resin"; copolymers such as a copolymer of melamine formaldehyde and ethylene urea formaldehyde; and the resin known to the trade as Uron which has the formula



In addition to resins of the above type, one can suitably employ epoxy resins and specific examples of suitable resins of this class include the diglycidyl ether of ethylene glycol, the triglycidyl ether of glycerol, and the epoxy resin sold by Shell Chemical Company under the name of "Eponite 100." Still another class of resins which can suitably be employed are triazinone resins and any member of this type of resins coming within the above defined group can give satisfactory results according to the process of this invention. Still another resin which can be employed is tris (1-aziridinyl) phosphine oxide which is prepared by reacting 3 moles of ethyleneimine with 1 mole of  $\text{POCl}_3$  and which is known to the trade as "APO Resin" or "Imine I.P. Resin." One need not employ a single resin material but can employ blends of resins of the above type or copolymers where available. Likewise, it is not necessary that the resins be entirely free from water insoluble components since it has been found that dispersed particles of water insoluble materials in the resin solution are not deleterious even though any portion of the resin that is water insoluble does not contribute to the beneficial results obtainable according to this invention. Some of the commercially available resinous materials mentioned above contain small percentages of water insoluble polymeric materials

and while an aqueous mixture of such resins can be filtered if desired, equally satisfactory results are generally obtained by employing the unfiltered material.

Suitable acid catalysts for resins of the above types are well known in the art. Urea formaldehyde and melamine formaldehyde resins are best catalyzed by chloride or nitrate salts of hydroxylalkyl amines such as monoethanol amine hydrochloride or 2 amino-2 methyl-propanol nitrate. Cyclic ethylene urea formaldehyde resins, acetylene diurea formaldehyde and Uron resins are preferably catalyzed by zinc nitrate or by magnesium chloride. The epoxy resins are preferably catalyzed by acid fluoride salts, such as the catalyst compositions available from Shell Development Company under the trade names of "Curing Agent 48" and "Curing Agent 20." The above catalysts are all characterized by their ability to furnish hydrogen ions which are necessary for the condensation or etherification reactions taking place during the curing cycle. Generally any amount of catalyst up to about 5% by weight of the solution will give satisfactory results with the preferred range being from about 0.5% to 2% by weight of the resin solution.

The amount of resin which is applied to the textile fabric according to this aspect of the invention can be varied within wide limits and the most advantageous amount is dependent upon a number of variables, especially the particular type of resin being employed. It is a general rule that the greater the degree of cross linkage, the smaller the amount of textile resin which can effectively be employed, and one can obtain results by employing only a relatively small amount of resin on a highly cross linked cellulosic fabric that is comparable to those obtained by employing a relatively larger amount of textile resin on a cellulosic fabric, the fibers of which are to be cross linked to only a slight degree. In most instances, it is desirable to employ only a small amount of the resin material and from 1% to 5% resin solids on the weight of the fabric generally gives optimum results. Due to the synergistic action of the cross linking agent and the textile resin, the effectiveness of the textile resin is greatly increased as compared to prior art procedures of resin applications to cellulosic fabrics and satisfactory minimum care characteristics and wrinkle resistance can sometimes be obtained employing as little as 0.5% resin solids based on the weight of the fabric. At the other extreme, the amount of resin materials in some instances up to as much as 10% to 15% by weight of the fabric can be employed without imparting an unacceptable hand, but the addition of such large amounts of resin is generally not necessary and is not economically desirable.

A unique feature of this aspect of the invention when both cross linking agent and textile resin are used is that both can be and are applied from the same aqueous solution containing the desired amount of textile resin, catalyst therefor, and cross linking agent (but without the catalyst for the cross linking agent). Conventional padding equipment is suitable for applying the solution and with such apparatus, the textile fabric can be passed through the aqueous solution to give sufficient solution pick-up by the fabric to provide the desired amount of resin solids and cross linking agent on the fabric. Following the application of the solution, the fabric is dried and heated to cure the resin. The most advantageous curing temperature depends upon the particular resin and catalyst employed. As a general rule, the curing temperature is a range from 100° C. to 200° C. and preferably between 150° C. and 180° C. The curing temperature should be maintained for from 10 seconds to 30 minutes with the preferred range being from 30 seconds to 5 minutes, depending upon the temperature, amount, and kind of material and the particular resin compound.

After the textile resin has been cured, the fabric, still containing the uncured cross linking agent, is treated with alkaline catalyst to bring about the reaction between the functional groups of the cross linking agent and the cellu-

lose hydroxyl groups as described above. The strong alkaline catalyst, several types of which have been mentioned previously, may be applied by known techniques including the padding technique used for applying the resin and the cross linking agent.

The amount of sulfato sulfone cross linking agent may be varied within relatively wide limits, but the amount will generally be somewhat smaller than that used without the resin. In most instances, 0.005 moles of cross linking agent per anhydro-glucose unit will be sufficient to give the product noticeably flat drying, wet crease resistance, and wet configurational memory. Best results are generally obtained when the fabric is reacted with 0.01 to 0.02 mole of cross linking agent per anhydro-glucose unit. Amounts of the agents greater than 0.03 mole per anhydro-glucose unit are generally avoided because it may produce excessive stiffness and degradation of the fiber.

The important advantages of the invention are attributable to the fact that both the resin and the sulfato sulfone cross linking agents are present in a single solution that is applied to the fabric in one step. At the time the resin is being cured with catalyst, the cross linking agent remains unaffected because it is nonvolatile and nonreactive in acid medium. However, it is still present on the fibers and still in immediate contact with the fibers and therefore in a position where it can exert its effect when the proper conditions are present. Furthermore, it is believed that the cross linking agent may react with some of the active hydrogens of the resin. Wet slickness and excessive hydrophobic properties have been attributed to the presence of too many active hydrogens, and hence the removal of some of them by the cross linking agent is desirable.

After the resin has been cured, the alkaline conditions are produced to cure the cross linking agent. Such alkaline conditions would normally have a bad effect on the resin, but because the resins have been cured, they are not harmed under the controlled conditions and limited time of exposure that are maintained to cure the cross linking agent.

The invention will now be described more specifically in terms of examples in which all parts are by weight unless otherwise indicated.

#### Example I

*Preparation of the sulfide.*—The sulfide is a known material available on the market. It was prepared by introducing gaseous ethylene oxide and hydrogen sulfide in the proportion of 2 moles of the former to 1 mole of the latter into the bottom of a packed column containing a small amount of the reaction product to initiate the reaction. The exothermic reaction took place in the column to form the sulfide, which flowed down through the column and was withdrawn.



The reaction in the column took place at about 45° C. to 60° C. The yield was about 95% to 100% of the theory.

In a similar way using known procedures, substituted ethylene oxides (which are liquids) can be used to prepare substituted sulfides by reaction with H<sub>2</sub>S as follows



*Preparation of the sulfoxide.*—Bis(hydroxyethyl sulfide, for example (HO-CH<sub>2</sub>-CH<sub>2</sub>)<sub>2</sub>S, which is a liquid, is diluted with water in the proportion of about 500 parts of the sulfide to 200 parts of water. The mixture is

5

cooled in an ice bath and stirred while adding 30% hydrogen peroxide. About 1.2 moles of peroxide are added per mole of sulfide. The reaction is strongly exothermic but the temperature is kept below 65° C. by stirring and cooling. The corresponding sulfoxide



is formed in about 95% to 100% yield.

*Preparation of the sulfone.*—After all of the peroxide needed for the preparation of the sulfoxide has been added, the mixture is heated and refluxed at the pot temperature of 100° to 110° C. Another mole of 30% H<sub>2</sub>O<sub>2</sub> is added slowly while continuing the refluxing. The pot temperature will increase somewhat above 110° C. After all peroxide has been added, refluxing is continued for two to five hours to decompose excess peroxide. The end point is determined by carrying out starch-iodine tests. Water is then evaporated under vacuum to give the sulfone in a yield of 90% to 95%, i.e., about 600 parts of the sulfone (HO-CH<sub>2</sub>-CH<sub>2</sub>)<sub>2</sub>SO<sub>2</sub>. These compounds are also known.

*Preparation of the bisulfatoethyl sulfone.*—Thirty percent fuming H<sub>2</sub>SO<sub>4</sub> is added to the sulfone, which is a viscous oil, with cooling and stirring. 2.2 moles of SO<sub>3</sub> (including free SO<sub>3</sub> and the SO<sub>3</sub> equivalent of the H<sub>2</sub>SO<sub>4</sub> present) are used per mole of the sulfone. The reaction is exothermic and it is preferred to hold the temperature in the range of about 5° to 10° C. during the addition. Thereafter the mixture is allowed to come to room temperature, where it is kept about two to four hours. With cooling and stirring to maintain a temperature below 20° C. the mixture is poured into an equal volume of water. The product at this point has the structure



The acid form of the bisulfatoethyl sulfone can be used as such as a cross linking agent for treating cellulosic fibers following the same procedure described above, or it can be converted to the metal salt.

*Preparation of the metal salt.*—In making the sodium salt, sodium hydroxide or preferably sodium carbonate is added in amount sufficient to replace all of the acid hydrogens of the sulfatoethyl groups. Sodium sulfate precipitates at the high concentration of sodium ion prevailing and can be filtered off. The yield of the sodium salt is about 50% based on the sulfone. To get the solid sodium salt, water is evaporated under vacuum until the liquid in the pot begins to solidify. The pot is cooled and the material is recrystallized from a solution of 25% water and 75% acetone by volume. An alternative procedure is to evaporate until the liquid slurry is present in the pot. Acetone is then added to the slurry in the pot to precipitate the desired sodium salt. The impurities are mainly retained in the solution.

The product contains the ion



in association with positive, e.g., metallic ion or ions. The product having the chemical formula



exists as a monohydrate having a melting point of 162° C. and as a non-hydrated material having a melting point of 141.5° C., both of which are white crystalline solids. More generally, the materials in which the ethylene hydrogens may be substituted with alkyl groups having 1 to 3 carbon atoms are described by the structural formula:



## 13

where "Me" refers to positive ions having two valences matched by the divalent bisulfatoethyl sulfone anion. The divalent anion is believed to be present as described in the structural formula irrespective of the particular cation associated therewith and irrespective of whether the compound is in the form of a liquid, a solid, or in solution.

*Treatment of cloth.*—A 15% aqueous solution of the bisulfatoethyl sulfone sodium salt or other metal salts is fed to padding rolls while the cotton cloth to be treated (4 yards 80 x 80) is passed downwardly between the rolls. The amount of solution supplied is sufficient to give 75% liquid pick-up by the cloth. The fabric is then dried, preferably at room temperature, after which it is again padded with 2% aqueous sodium hydroxide solution saturated with sodium chloride (to retard any tendency of the sulfone to go into solution). The caustic padded cloth is held at room temperature for one hour, then washed thoroughly with detergent, rinsed, and dried. The finished fabric has the desired flat drying qualities while retaining a high degree of strength. It also has wet crease resistance and configurational memory.

## Example II

The procedure of Example I is carried out except that the fabric is treated with the bisulfatoethyl sulfone and dried, then immersed in 2% aqueous sodium hydroxide saturated with sodium chloride at 40° C. for thirty seconds. It is then removed, washed thoroughly with a detergent, rinsed and dried. The fabric obtained has the desirable flat drying and other qualities substantially like the product of Example I.

## Example III

A 21% by weight solution of the compound



in water is prepared and is padded on a viscose rayon fabric having a count of 97 x 51 and a weight of 6.5 oz. per yard and made of 19.8/1 warp and 19.8/1 filling of spun viscose staple fiber, to give a pick-up of 70% by weight of the solution based on the weight of the unpadded fabric. It is air dried and then padded again with 2% aqueous sodium hydroxide solution saturated with sodium chloride at room temperature. The pick-up of aqueous sodium hydroxide solution is also 70%. The fabric is rolled up into a roll and wrapped in aluminum foil where it is left for one hour at room temperature. The fabric is thereafter washed thoroughly with detergent in hot water, rinsed, and dried. The finished fabric has good flat drying properties, wet crease resistance, and wet configurational memory.

## Example IV

A 13% by weight of aqueous solution of the compound



is prepared and is padded on woven cotton fabric (4 yard 80 x 80) according to the procedure described in the previous examples. The pick-up of solution by the fabric is also 70%. The fabric is dried in the air and is repadded with 2% aqueous sodium hydroxide saturated with sodium chloride to a pick-up of 70%. The fabric is immediately rolled and wrapped in aluminum foil and stored for one hour at room temperature and is thereafter unrolled and washed thoroughly in hot water containing a detergent, rinsed, and dried. The product has good flat drying properties, wet crease resistance, and wet configurational memory.

## 14

## Example V

A 28% by weight aqueous solution of the compound

5



10

is prepared and is padded on a cotton fabric (4 yard 80 x 80) to give a solution pick-up of 70% by weight. The fabric is air dried and then immersed in a 2% aqueous NaOH solution without sodium chloride at 70° C. for about 15 seconds. It is then withdrawn and immediately washed thoroughly with hot water containing detergent, rinsed, and allowed to dry in the air. The fabric has good flat drying properties, wet crease resistance, and wet configurational memory.

15

## Example VI

A 24% by weight aqueous solution of the compound

20



25

is prepared and is padded on a cotton fabric to get a 70% pick-up of solution, after which it is dried in the air. It is then immersed in a 5% aqueous NaOH solution saturated with sodium chloride at 35° C. for sixty seconds. At the end of that time, it is withdrawn, washed thoroughly in hot water containing a detergent, rinsed, and dried in the air. The fabric has good flat drying properties, wet crease resistance, and wet configurational memory.

30

## Example VII

A 9% aqueous solution of the compound

35



is prepared and is padded on a cotton fabric to give a 70% pick-up of the solution by the fabric, after which it is dried in the air. It is then repadded with a 3% aqueous NaOH solution saturated with sodium chloride, again to give a wet pick-up of 70%. The fabric is then rolled up, wrapped in aluminum foil and stored at room temperature for one hour. Thereafter, it is unrolled, washed thoroughly in hot water containing a detergent, rinsed, and allowed to dry. The fabric has good flat drying properties, wet crease resistance, and wet configurational memory.

50

## Example VIII

55 A 16% aqueous solution of the compound



is prepared and is padded on a 4 yard 80 x 80 cotton fabric. It is then immersed in a 3% aqueous solution of 60 benzyl trimethyl ammonium hydroxide at 50° C. for 45 seconds, after which it is withdrawn and immediately washed thoroughly with hot water containing a detergent. The fabric is rinsed, dried and found to have good flat drying properties.

65

## Example IX

An aqueous solution consisting of 10% of the sulfato sulfone

70

75 10% Aerotex 23 (containing 50% solids) a modified melamine formaldehyde resin sold by American Cyanamid Company, 0.8% zinc nitrate (catalyst), 6% Moropol 700 (emulsified polyethylene softener) made by Mortex Chemical Products, Inc. containing 30% solids is then padded



onto a cotton fabric to give 70% pick-up based on the weight of the fabric. The infrared absorption spectrum of Aerotex 23 is shown in FIGURE 1. It is then air dried and cured at 160° C. for one and one-half minutes. The fabric is then immersed in 2% aqueous sodium hydroxide saturated with sodium chloride at 35° C. for 30 seconds. It is immediately withdrawn and washed in hot water containing detergent, rinsed, and dried. The fabric has crease resistance comparable to fabrics treated with twice the amount of the same resin without cross linking agent. The wet crease resistance and the wet configurational memory are comparable to a fabric that has been treated with a larger amount of the same cross linking agent, but without resin.

Although this aspect of the invention has been illustrated in terms of using a specific sulfato sulfone as cross linking agent, the same effects could be obtained with any of the other cross linking agents described above.

The foregoing description has been directed to the use of sulfones as cross linking agents. Another group of cross linking agents having similar properties are the sulfoxides, which are represented by the same general structural formula



except that the group X is  $-SO-$  or  $-SO-R-SO-$ . The counterpart of the cyclic sulfone cross linking agent is



In all of the structural formulae for the sulfoxide cross linking agents, the same symbols R<sup>1</sup>, R<sup>2</sup>, and Y are defined in exactly the same way as they are in the case of the sulfone cross linking agents.

The effect of the sulfoxide group is believed to be substantially the same as the effect of the sulfone group described above, that is, it activates the sulfato group toward the cellulose hydroxyl groups to produce cross linking. Therefore, the reaction mechanisms and reaction conditions described above for the sulfone cross linking agent apply also to the use of the sulfoxide cross linking agents. Specifically, the molar proportions of the cross linking agent and the anhydro-glucose units, and the types and concentrations of strong alkali used during the cross linking reaction generally are the same for the sulfoxides and the sulfones. Furthermore, the sulfoxides can be used for cross linking the several types of cellulosic fibers (cotton, regenerated cellulose, chemically modified cellulose) that were described in connection with the sulfones.

The following is an example giving a specific procedure for cross linking cotton fibers with a sulfoxide cross linking agent.

#### Example X

The following sulfoxide was prepared as an intermediate in the preparation of the sulfone used in Example I.



The aqueous solution of the sulfoxide is evaporated to dryness under vacuum and the white crystalline product is obtained in a yield of 95% to 100% of theoretic, based on the sulfide. The sulfoxide is reacted with 30% fuming sulfuric acid in the ratio of 1 mole of sulfoxide to 3 moles of SO<sub>3</sub> (based on total free SO<sub>3</sub> and SO<sub>3</sub> equivalent to the H<sub>2</sub>SO<sub>4</sub>).

The fuming sulfuric acid is placed in a vessel equipped with a stirrer and surrounded by an ice bath. The sulfoxide is added in small amounts periodically over a period of three hours taking care that the temperature of the mixture does not go above 20° C. After all of the sulfoxide has been added, stirring is continued for two to four hours and the material is allowed to warm up to room temperature. The liquid reaction product is

added slowly to an equal volume of water while cooling it to keep the temperature below 20° C. It is then neutralized to a pH of seven by adding sodium carbonate. Due to the high concentration of the sodium ion, most of the sodium sulfate is precipitated and is removed by filtration. The product is evaporated to dryness under vacuum to obtain a white crystalline product in about 50% yield based on the bishydroxyethyl sulfoxide. The product has the following composition:



This is a new composition of matter and may be represented by the general structural formula



wherein the symbols have the same meaning as described thereto in discussing the sulfones.

*Treatment of cloth.*—A 25% aqueous solution of the bisulfatoethyl sulfoxide is prepared and padded onto a 4 yard 80 square cotton fabric to give a 70% by weight pick-up of the solution. It is air dried and then immersed in a 2% aqueous sodium hydroxide solution saturated with sodium chloride. The alkaline solution is at 70° C. Immersion is for 3½ minutes. The cloth is then withdrawn and immediately washed in a hot aqueous solution containing a detergent, rinsed, and dried at room temperature. The fabric has very good flat drying properties, wet crease resistance, and wet configurational memory.

Other sulfoxides that are effective in treating cellulosic fibers according to the invention are those that have the same structural formula as the compounds used in Examples I to IX, inclusive, and others described in the specification except that the sulfone group  $-SO_2-$  is replaced with the sulfoxide group  $-SO-$ .

#### Example XI

The fabric is prepared as in Example X and immersed in an aqueous 15% acetic acid solution containing metallic zinc, and is held at a temperature of 35° to 40° C. The treatment is continued for 15 minutes in order to reduce the sulfoxide (S—O) groups in the cross links to sulfide groups (S). The fabric is then withdrawn, washed thoroughly with hot water containing a detergent, rinsed, and dried in the air. The fabric still has substantially the same flat drying, wet crease resistance, and configurational memory properties, but the chlorine absorption is substantially reduced. Instead of using zinc and acetic acid to reduce the sulfoxide linkages between the cross linked cellulose chains, the reduction may be carried out in similar reducing media that do not cause decomposition of the cellulose. The advantage of being able to reduce the sulfur in the cross linkages applies to the other sulfoxide cross linking agents as well.

#### Example XII

An 80 x 80 4 yard cotton print cloth, bleached and mercerized, is treated with a solution containing 15% diglycidyl ether of tetraethylene glycol, 20% bis (sodium sulfatoethyl) sulfone, 1% zinc fluoroborate, and 64% water. The fabric is padded with the solution, dried and cured one and one-half minutes at 150° C. The cured fabric is then padded with 3% NaOH, rolled up damp and held at room temperature for 6 hours. The cloth is then washed and dried. It has excellent line and tumble drying properties.

#### Example XIII

A cotton fabric, bleached and mercerized, is treated with a solution containing 10% HCHO, 20% bis (sodium sulfatoethyl) sulfone, 1% oxalic acid and 69% water.

The fabric is padded with the above solution, dried and cured two minutes at 150° C. The cured fabric is then padded with 3% NaOH, rolled up at room temperature and aged six hours. The fabric is then washed and dried. It has excellent line and tumble drying properties.

Having thus described my invention and several embodiments thereof, what I desired to claim and secure by Letters Patent is:

1. The compound



wherein R<sup>1</sup> and R<sup>2</sup> are selected from the group consisting of hydrogen and alkyl groups having one to three carbon atoms and wherein Me<sup>++</sup> represents positive ions having two valences matched by the divalent bis(sulfoalkyl) sulfoxide anion.

2. The compound



References Cited by the Examiner

UNITED STATES PATENTS

- |           |        |                        |         |
|-----------|--------|------------------------|---------|
| 1,422,869 | 7/1922 | Kranzlein et al. ----- | 260—458 |
| 1,968,926 | 8/1934 | Berthold et al. -----  | 260—607 |

|              |         |                        |           |
|--------------|---------|------------------------|-----------|
| 2,140,569    | 12/1938 | Ufer et al. -----      | 260—607   |
| 2,204,976    | 6/1940  | Van Peski et al. ----- | 260—458   |
| 2,335,119    | 11/1943 | Hoeffelman -----       | 260—458   |
| 2,524,399    | 10/1950 | Schoene et al. -----   | 8—116     |
| 5 2,645,659  | 7/1953  | Morris et al. -----    | 260—458   |
| 2,670,265    | 2/1954  | Heyna et al. -----     | 8—49      |
| 2,785,947    | 3/1957  | Kress -----            | 8—116     |
| 2,988,417    | 6/1961  | Emmons et al. -----    | 8—116     |
| 3,000,762    | 9/1961  | Tesoro -----           | 117—139.5 |
| 10 3,046,075 | 7/1962  | Kanter -----           | 8—17      |

OTHER REFERENCES

- Dyer & Textile Printer, April 20, 1962, p. 570.  
 Keller, Ind. & Eng. Chem. Nov. 1963, pp. 12, 13.  
 15 Nature, Oct. 25, 1958, vol. 182, pp. 1164—1165; 167—  
 78c—anti-metab.  
 Reichstein et al., Chem. Abstracts, vol. 30 (1936),  
 col. 6384.  
 Steinkopf et al., Ber. Deut. Chem., vol. 53 (1920),  
 20 pages 1007—1009.  
 Stahmann et al., J. Org. Chem., vol. 11 pp. 719—722,  
 729—731, 735.

LORRAINE A. WEINBERGER, Primary Examiner.

25 MORRIS O. WOLK, LEON ZITVER, Examiners.